

Aug. 18, 1942.

C. G. FINK ET AL

2,293,248

ELEMENT FOR PHOTOCELLS AND RECTIFIERS

Original Filed Aug. 10, 1940

Fig 1



Fig 2



INVENTORS  
COLIN G. FINK  
EDWARD ADLER

BY

Gustav R. Thompson  
ATTORNEY

## UNITED STATES PATENT OFFICE

2,293,248

ELEMENT FOR PHOTOCELLS AND  
RECTIFIERSColin Garfield Fink and Edward Adler,  
New York, N. Y.Continuation of application Serial No. 352,134,  
August 10, 1940. This application June 10,  
1941, Serial No. 397,404

12 Claims. (Cl. 175—366)

This invention relates to elements for photocells and rectifiers having light sensitivity and asymmetrical conducting electrical properties, and to the method of manufacture thereof; and provides improvements therein.

Elements of the solid, cuprous oxide, type, for photocells and rectifiers have heretofore been used.

It has also heretofore been proposed to increase the light sensitivity of such elements. For example, according to Fink and Fogle, Transactions of the Electrochemical Society, vol. 66, page 305, the photo-activity of such elements may be increased by subjecting the surface of the cuprous oxide to an acid etch, using solutions of nitric acid, hydrochloric acid, etc. Another method is to sensitize the surface of the cuprous oxide by ionic bombardment in a glow-discharge.

Cuprous oxide elements sensitized by previously known methods deteriorate or age rather quickly. Muller and Teeters, Trans. Electrochemical Society, vol. 69, page 467, reported that, after fifteen minutes, following sensitization by sputtering in a glow-discharge, the output of a cuprous oxide photocell dropped from an initial value of 570 microamperes to 275 microamperes. The ageing, accompanied by decrease in photo-activity continued throughout the life of the cell, although more slowly after the sharp initial drop in activity. Muller and Teeters attributed the deterioration to a reaction between one of the atmospheric constituents, such as oxygen, or carbon dioxide, and the sensitized surface at the interface between the cuprous oxide and the front electrode.

Similarly the elements, when used for rectifying alternating current, do not have the desired stability, and age, or lose efficiency in a relatively short time.

The present invention provides a new and improved method of increasing the sensitivity or output of a photoelectric element of the cuprous oxide type. The invention further provides an element of the type described having an improved output or sensitivity, improved electrical conductivity at the junction between the cuprous oxide layer and the front electrode, and improved stability and resistance to deterioration due to handling, ageing, ordinary use, or to harmful interaction with certain atmospheric constituents.

The invention further provides a rectifier element of the type described having an improved electrical conductivity and electrical contact at the junction between the cuprous oxide layer

and the front electrode, and improved stability and resistance to deterioration due to handling, ageing, ordinary use, or to harmful interaction with certain atmospheric constituents.

5 The invention further provides an element of the type described in which the leakage of current, when the element is used for rectification, in the reverse or high resistance direction is reduced.

10 Embodiments of the invention are illustrated in the accompanying drawing, wherein:

Fig. 1 is a diagrammatic cross-section, of an element according to the present invention, with adaptations for use as part of a photo-electric cell.

Fig. 2 is a view similar to Fig. 1 illustrating the element with adaptations for use in an apparatus for rectifying alternating current.

15 The present invention is based upon our discovery that by exposing the surface of cuprous oxide for a limited time to the action of moist hydrogen sulfide gas, or by dipping or brushing the surface of cuprous oxide with a solution of a sulfide, such as hydrogen sulfide, sodium sulfide, etc., the several advantages hereinbefore set forth are obtained.

20 In addition to simple sulfides, soluble polysulfides may also be used; and also substances which react to form sulfides. Examples of such substances are sodium polysulfide, sodium thiosulfate, an alkaline solution of thiourea, etc.

25 While sulphur vapor produces to a limited extent the results of the present invention, when the temperature of the gas does not exceed 100° C., the other modes of producing the cuprous sulfide film are much preferred, as the results are much superior, and the procedure much simpler.

30 The improved results of the present invention are also obtained with the other members of the sulphur group, i. e. selenium and tellurium. For example, gaseous selenides, tellurides, solutions of selenides or tellurides, and solutions yielding such selenides or tellurides, give results similar to those obtained when sulphur and its compounds are used.

35 The method is carried out by subjecting the cuprous oxide, in one of a number of ways, to the action of an element of the sulphur group or their compounds. This may be done by subjecting the cuprous oxide to the action of a gas or vapor of a compound of the element, or to a solution of an appropriate compound of an element of the sulphur group. According to our experience the best results are obtained when dilute solutions are used. One percent solutions

have been found to be effective. Generally it is preferable to use a solution of a soluble sulfide such as sodium sulfide. When the cuprous oxide is treated in or with a solution it is afterwards rinsed in water and dried.

When subjected to the action of a compound of sulphur, there is formed on the surface of the cuprous oxide a very thin and adherent grayish film of cuprous sulfide ( $Cu_2S$ ); and similar films are formed when compounds of the other elements of the sulphur group are used.

After the element has been sensitized as previously described, it is adapted or modified for use in a photo-sensitive apparatus, or in a current rectifying apparatus, in any suitable or well-known manner.

Referring to Fig. 1, numeral 10 designates a sheet of copper, having a layer 12 of cuprous oxide thereon. The cuprous oxide may be formed on the copper 10 by thermal oxidation, or by electrodeposition, according to known methods. Numeral 14 designates the thin film of cuprous sulfide which is formed when the cuprous oxide layer 12 is subjected to the action of a compound of an element of the sulphur group, according to the method herein described. When selenium or tellurium compounds are used, the film 14 is copper selenide or copper telluride. On the face of the element in contact with the copper sulfide film there is a front electrode 16, which is here shown as a pressed-on metallic grid. Alternatively, a front electrode may be applied by spraying, evaporating, or sputtering on to the surface 14 a translucent metal film.

Referring to Fig. 2 the parts 10, 12 and 14 have the same structure and composition as they have in the element of Fig. 1. A front electrode is provided by applying a sheet of metal 18, advantageously lead or tin, to the film 14.

Conducting wires are attached to the copper sheet 10 (back electrode) and to the front electrode or grid 16, Fig. 1. In Fig. 2 the electrical connections are made to copper sheet 10 (back electrode) and to the lead or tin sheet 18 (front electrode).

The increase of photo-electric sensitivity of elements produced according to the present invention is shown by the following comparison. At an illumination intensity of 2000 lux, with 8 square centimeters of surface exposed, an untreated cuprous oxide cell generated a photo-current of 3.0 microamperes. The element is then dipped in a 1% solution of sodium sulphide for 20 seconds, rinsed and air-dried. This results in the formation on the cuprous oxide surface of a very thin, adherent, grayish film of cuprous sulfide ( $Cu_2S$ ), having a thickness on the order of 400 Angstrom units, or 0.000004 centimeter. The element, after the aforesaid treatment, under the same conditions of illumination and measurement as before, generated a photo-current of 300 microamperes, an increase of one hundred fold, or ten-thousand percent. This we explain in part by the fact that, while the specific resistance of  $Cu_2S$  (cuprous sulphide) is greater than that of  $Cu_2O$  the nature of the  $Cu_2S$  surface is such that the conductivity across the meeting faces of the  $Cu_2S$  and the front electrode 16 (air-gap) is greatly improved, and also because of the presence of a greatly increased number of photo-active centers.

An advantage offered by the sensitization process of the present invention is that photo-cells so sensitized have an increased stability and

photo-activity over a relatively long period of time and do not suffer appreciable deterioration due to ordinary handling, use, ageing, or to harmful interaction with the atmospheric constituents.

The increased stability and freedom from deterioration of elements according to our invention may be explained by the adherent film of copper sulfide (or telluride or selenide) produced by our method. These substances (copper sulfide, copper selenide, copper telluride) are relatively stable, especially in city atmospheres, being not readily susceptible to oxidation by the oxygen of the atmosphere, or to interaction with carbon dioxide of the air. In previous sensitizing processes, the photo-sensitive surface was thought to comprise freshly reduced copper (see Muller and Teeters loc. cit. p. 471; also B. Lange "Photoelements" I. (Barth, Leipzig) p. 34 (1936); freshly reduced copper is known to be chemically active and would readily react with the oxygen or carbon dioxide of the atmosphere, with a consequent decrease in photo-activity.

Another advantage offered by the present invention lies in the fact that the adherent, active, film of copper sulfide (or copper selenide or telluride) improves the electrical conductivity between the cuprous oxide layer and the "front" electrode connecting the photocell to an external circuit, and also provides a good and stable electrical contact between the cuprous oxide layer and the "front" electrode, thereby increasing the efficiency and stability of the photocell. There are the same advantages when the element is used in a rectifier. The rectifying apparatus is more efficient, and has greater stability than heretofore, when equipped with an element according to the present invention. In rectifiers it is important, in order to obtain good operating efficiency and to minimize the amount of heat developed in operation, that good electrical conductivity and good electrical contact be maintained between the cuprous oxide layer of the rectifier and the front electrode. These good properties are obtained according to our invention by the cuprous sulfide film between the cuprous oxide and the "front" electrode.

The improvement in efficiency of photo-sensitive cells and of rectifiers, resulting from our invention persists over long periods of time, thus providing a stability of operation in prolonged use which has been hitherto unobtainable from photocells or rectifiers of the cuprous oxide type. Photo-sensitive cells provided with elements made according to the present invention have been under test for three-month periods with a decrease of efficiency of less than 10%.

This application is a continuation of our application Serial No. 352,134, filed August 10, 1940.

What is claimed is:

1. An improved element for photocells and rectifiers, having light-sensitive and asymmetrical conducting electrical properties, comprising cuprous oxide and a thin film having a thickness on the order of 400 Angstrom units consisting of a compound of copper and an element of the sulphur group on the cuprous oxide.
2. An improved element for photocells and rectifiers, having light-sensitive and asymmetrical conducting electrical properties, comprising cuprous oxide and a thin film having a thickness on the order of 400 Angstrom units consisting of cuprous sulfide on the cuprous oxide.
3. An improved element for photocells and rectifiers, having light-sensitive and asymmetrical

conducting electrical properties, comprising cuprous oxide and a thin film having a thickness on the order of 400 Angstrom units consisting of copper selenide on the cuprous oxide.

4. An improved element for photocells and rectifiers, having light-sensitive and asymmetrical conducting electrical properties, comprising cuprous oxide and a thin film having a thickness on the order of 400 Angstrom units consisting of copper telluride on the cuprous oxide.

5. A method of making improved elements for photocells and rectifiers having light-sensitive and asymmetrical conducting electrical properties, comprising exposing the cuprous oxide portion of such an element to the action of an element of the sulphur group or a compound thereof only long enough to form a film having a thickness on the order of 400 Angstrom units.

6. A method of making improved elements for photocells and rectifiers having light-sensitive and asymmetrical conducting electrical properties, comprising exposing the cuprous oxide portion of such an element to the action of sulphur or a compound thereof only long enough to form a film having a thickness on the order of 400 Angstrom units.

7. A method of making improved elements for photocells and rectifiers having light-sensitive and asymmetrical conducting electrical prop-

erties, comprising exposing the cuprous oxide portion of such an element to the action of selenium or a compound thereof only long enough to form a film having a thickness on the order of 400 Angstrom units.

8. A method of making improved elements for photocells and rectifiers having light-sensitive and asymmetrical conducting electrical properties, comprising exposing the cuprous oxide portion of such an element to the action of tellurium or a compound thereof only long enough to form a film having a thickness on the order of 400 Angstrom units.

10 9. A method according to claim 5, wherein the element or its compound is in the form of a solution to which the cuprous oxide is exposed.

15 10. A method according to claim 5, wherein the element or its compound is in the form of a gas or vapor to which the cuprous oxide is exposed.

11. A method according to claim 5, wherein the element or its compound is in the form of a dilute solution of a sulfide or of a compound which reacts to form a sulfide, to which the cuprous oxide is exposed.

12. A method according to claim 5, wherein the element or its compound is in the form of a sulfide gas to which cuprous oxide is exposed.

COLIN GARFIELD FINK.  
EDWARD ADLER.